

Oct. 5, 1937.

N. E. COOK ET AL

2,094,583

MANUFACTURE OF METAL COATED PRODUCTS

Filed March 22, 1935



INVENTORS

Nelson E. Cook  
Edward J. Knott  
William L. Diele  
By \_\_\_\_\_, Seal, S. C. \_\_\_\_\_

## UNITED STATES PATENT OFFICE

2,094,583

MANUFACTURE OF METAL COATED  
PRODUCTS

Nelson E. Cook, Wheeling, W. Va., Edward J. Knopf, Morristown, Ohio, and William L. Diehl, Wheeling, W. Va., assignors to Wheeling Steel Corporation, Wheeling, W. Va., a corporation of Delaware

Application March 22, 1935, Serial No. 12,398

6 Claims. (Cl. 91—70.2)

This invention relates to the manufacture of metal coated products, and, while not specifically so limited, has particular application in the coating, and especially the galvanizing, of sheet metal, 5 such, for example, as steel sheets. Superior coated products, and particularly galvanized sheet steel products, are produced. Such products are claimed in our copending application Serial No. 54,278, filed December 13, 1935, which 10 application is in part a division of this application. This application is in part a continuation of our copending application Serial No. 741,222, filed August 24, 1934.

Purely for purposes of description and illustration the invention will be described as applied to the manufacture of galvanized or zinc coated steel sheets. Sheets of this character have wide commercial use. As ordinarily made they have both sides spangled,—that is, the zinc coating in 20 cooling forms over both surfaces of the sheet large heterogeneous crystals or spangles readily distinguishable to the naked eye even at some distance. For most purposes these spangled surfaces are not undesirable, and indeed they are 25 definitely desirable in cases where a certain type of finished appearance is wanted.

However, for other purposes sheets having both surfaces spangled are definitely undesirable, as, for example, when the product is to be painted. 30 Spangled galvanized surfaces will not take paint readily. It has been the practice heretofore to permit spangled galvanized sheets to weather, or to artificially weather them, as by treatment with acid or other chemical having the effect of 35 oxidizing the surfaces of the sheets, in order that the surfaces to be painted may become somewhat roughened so that paint will readily adhere thereto.

We have discovered that galvanized sheets may 40 be produced without the ordinary spangled surfaces, without the undesirable buckling of the sheets which has attended previous efforts to produce unspangled galvanized sheets, and with a smooth dull matte or slightly roughened surface which is at the same time highly resistant 45 to corrosion, beautiful in appearance and readily receptive to paint and other similar coating materials. We are well aware of the previous efforts which have been made along these lines in 50 both the practical and the patented art, but no process having the features and advantages of our process has heretofore been proposed and no finish having the desirable qualities of our finish has heretofore been produced.

55 Before proceeding to explain our invention we

wish it understood that we do not claim broadly to have invented the formation of unspangled galvanized metal surfaces, as unspangled surfaces have been produced before. One way in which unspangled galvanized surfaces have been produced is by dipping the hot galvanized ware as it comes from the galvanizing pot into a liquid bath, which prevents the formation of spangles, produces a mottled, irregular, partly bright and partly dull surface and results in warping the ware due to the rapid and uneven temperature changes brought about by the dipping. The warping can be reduced to some extent by heating the bath in which the ware is dipped, but, aside from the question of warping, the finish is unsatisfactory in appearance, is not highly resistant to corrosion and will not take paint readily. It has also been proposed to subject galvanized ware to the action of a jet of water or other liquid, but this has substantially the same results as dipping. The finish produced is not uniform, being partly bright and partly dull and mottled, is not highly resistant to corrosion and will not take paint satisfactorily. Furthermore, the subjecting of the hot galvanized ware to a jet of liquid results in warping of the ware as in the case of dipping.

After considerable experimenting we have discovered that the highly desirable unspangled, uniform, dull matte finish may be produced by 30 subjecting the galvanized ware (here considered for purposes of illustration as comprising sheets) to the action of a mist or very fine spray. The mist or very fine spray is to be clearly distinguished from the jet of liquid referred to above, 35 as the results obtained by the two processes are entirely different. The sheets after leaving the galvanizing bath are brought into the presence of the mist or very fine spray before the large spangles characteristic of ordinary galvanized ware have formed. Almost immediately upon leaving the galvanizing bath the zinc coating begins to cool and crystallization commences. If this crystallization is allowed to progress unhindered the large spangles characteristic of ordinary galvanized ware will be produced. By bringing the hot sheets into the presence of the mist or very fine spray we prevent the formation of the large spangles and the desired uniform dull matte finish results.

While we are not certain as to the theory underlying the process above described, we think that the fine particles of the mist exert a physical effect on the surface of the sheet, creating relatively very closely spaced centers of propaga- 50

tion or crystallization from which the crystals form. But when the centers of propagation of crystals are relatively closely spaced the crystals are of relatively small size as adjacent crystals 5 during propagation come in contact with each other before the crystals can attain relatively large size, resulting, as it were, in the squeezing into the same surface area of a relatively very great number of relatively very small crystals 10 which, due to the relative proximity of their centers of propagation or crystallization, have had no opportunity to grow to or even to approach the size of what are commonly known as "spangles", which are readily distinguishable to 15 the naked eye even at some distance and which may in some cases extend from their respective centers of crystallization for a distance of an inch or more in various directions. If the size of the crystals is properly controlled the sheet will appear 20 to the naked eye to have a uniform continuous dull matte surface. Under a powerful magnifying glass this surface will be seen to be crystalline, presenting an appearance similar to an ordinary spangled surface. However, the relatively great number of relatively small, relatively closely spaced crystals affords an ideal surface for the reception of paint and similar coatings, and this surface is also particularly well suited for various uses without painting or covering with similar coatings, as, for example, for 25 oven linings.

We have found that by appropriately controlling the mist or spray and the passage of the sheet in relation thereto we can form a sheet 30 having one side spangled in the characteristic manner and the other side provided with the uniform dull matte finish above described. Sheets of this character are highly desirable and useful. For example, they may be used for signs, such as 35 advertising and highway direction signs, paint being applied to the side provided with the dull matte finish to form the front of the sign, and the back of the sign being left unpainted. The ordinary spangled finish of the back of the sign 40 effectively withstands corrosion so that a highly satisfactory yet relatively inexpensive sign is thus produced. Another use to which sheets having one side spangled in the usual manner and the other side provided with the uniform dull 45 matte finish may be put is in the construction of refrigerator cases. The side having the dull matte finish forms the outside of the case and receives the usual white enamel paint, while the spangled side faces toward the interior of the refrigerator and is naturally well adapted to withstand 50 corrosion due to moisture within the refrigerator. Sheets of this character may also be used for oven linings, the unpainted dull matte finish facing the interior of the oven.

Various materials may be used for producing the mist or very fine spray. Plain water alone if sufficiently finely divided is fairly satisfactory. Using a fine mist of plain water does not, however, give as exact control of surface appearance 55 as is desirable for many purposes. However, we have found that water solutions of certain chemicals produce markedly superior results. A few of the chemicals thus used listed approximately in the order of efficacy are copper sulphate, 60 sodium nitrate, sodium chloride, potassium chromate and potassium permanganate. These salts are precipitated rapidly from their water solutions at temperatures slightly above the solidifying point of zinc or the zinc alloys usually employed for galvanizing. The solidifying point of

the galvanizing material may be in the neighborhood of 760° F. to 800° F. While we are not certain as to the theory of action, we believe that the rapid evaporation of the water results in the almost immediate precipitation or deposition on the surface of the sheet of microscopic, almost unmeasurably small particles of the salt or of some precipitate formed upon the application of heat to the mist composed of the salt solution. This precipitate seems to have the effect of controlling the centers of propagation of the crystals so that such centers are distributed quite uniformly over the surface of the sheet and very close together. Apparently those substances whose 15 solutions most quickly deposit their precipitates on the surface of the sheet upon the application of heat in the neighborhood of the temperatures mentioned above are most satisfactory for our purpose.

Care must be taken to keep the mist very finely divided. If a relatively coarse spray or jet is used the sheet will either appear spangled or it will have a non-uniform mottled appearance, being partly bright and partly dull, and the surface will not be as suitable for painting as is the uniform dull matte surface produced by our process.

Other features, details, objects and advantages of the invention will become apparent as the following description of certain present preferred methods of treatment of coated sheets and certain present preferred apparatus for carrying out the method and producing the desired product proceeds.

In the accompanying drawing we have shown 35 certain present preferred forms of apparatus for producing coated sheets, in which

Figure 1 is a plan view of one form of apparatus;

Figure 2 is an elevational view, partly in vertical longitudinal cross section, of the apparatus shown in Figure 1; and

Figures 3 and 4 are each a detail elevational view, partly in vertical longitudinal cross section, of a portion of a modified form of apparatus.

The steel sheets which are to be coated are first treated to remove dirt and scale, as, for example, by pickling, blasting, etc. This step may be omitted if the sheets are originally clean. The sheets are then treated in apparatus as 50 shown in the drawing and now to be described.

Referring now more particularly to Figures 1 and 2, a set of feed rolls 10 is located adjacent the entrance of a galvanizing pot 11 of known construction and provided with entry guides 12 and feed rolls 13 by which sheets advancing through the feed rolls 10 are directed downwardly into the pot 11 through a flux bath 14 floating on the surface of the molten zinc or spebler contained in the pot 11. Guides 15 direct the sheets 60 through the spebler between bottom rolls 16. Guides 17 extend from the rolls 16 upwardly toward the exit rolls 18. As the sheets pass between the rolls 18 they are engaged by exit guides 19 which deliver them onto a conveyor 65 20 or other transporting means.

When the form of apparatus shown in Figures 1 and 2 is used the sheets are subjected to a mist or very fine spray as they are carried along by the conveyor 20. The mist or spray is indicated in Figure 1 by reference numeral 21 and is created by means of very finely adjusted spray nozzles 22 connected with a supply of the fluid being sprayed and a suitable source of spraying pressure. The position of a sheet on the con- 75

veyor 20 is indicated at 23. With this form of apparatus the spray impinges on both sides of the sheet. The nozzles may, however, be so positioned as to direct the spray against one or both sides of the sheet. The effect of the mist or fine spray is as explained above, resulting in the production of a dull silvery or matte finish in which the crystals are so small as not to be individually distinguishable by the naked eye.

10 The point at which the mist or spray impinges on the coated sheet may be varied within certain limits and the precise point at which the mist should impinge upon the sheet is dependent on various factors including the character and 15 temperature of the spelter, the speed of movement of the sheet, the width and thickness of the sheet, the weight of the coating, the factor of whether the mist is applied to one or both sides of the sheet, etc. It is, however, important that 20 the mist shall impinge upon the coated sheet before the process of crystallization has advanced far enough so that the production of crystals clearly distinguishable to the naked eye will result. As crystallization may not set in immediately upon delivery of the sheet from the spelter bath, particularly when a relatively heavy coating is applied, it is sometimes desirable not to treat the successive portions of the coated sheet with the mist until a predetermined time after 25 such portions have emerged from the spelter. For example, a treatment such as that above described and illustrated in connection with Figures 1 and 2 allows a relatively great time interval before treatment of the sheets with the mist, although, of course, the greater the speed of the sheets the greater the distance from the point of emergence of the sheets from the spelter to the point of impingement of the mist thereon may be.

40 The apparatus shown in Figure 3 is similar in all respects to that shown in Figures 1 and 2 except for the positioning of the nozzles 24. These nozzles are arranged in two series extending transversely of the sheet and substantially opposite each other in the direction of movement of the sheet, the nozzles being directed so that the mist impinges on the sheet at an angle in the direction of movement of the sheet. It has been found that when the nozzles are so positioned superior results are obtained. The reason for this is not definitely known although it is believed that when the nozzles are directed so that the mist impinges on the sheet at an angle in the direction of movement of the sheet the 45 effect is to more rapidly evaporate the mist particles without such a cooling effect as will produce spangles which may result if the nozzles are directed so that the mist impinges on the sheet at an angle in the direction opposite the direction of movement of the sheet. When it is desired to treat only one side of the sheet only one set of nozzles is operated, the other set being shut off. Also in Figure 3 the nozzles are spaced somewhat nearer the point of emergence of the 50 sheet from the bath than in Figures 1 and 2. However, the exact position of the nozzles relative to the point of emergence of the sheet from the bath may be varied as desired in accordance with the factors above mentioned.

55 In Figure 4, a further modified form of apparatus is disclosed, this apparatus likewise being the same as that of Figures 1 and 2 except for the positioning of the nozzles. In Figure 4 the nozzles 25 are positioned so as to spray laterally from one or both sides of the sheet, the spray

impinging both on the sheet and also on the exit rolls 18. An arrangement of this character is used on very thin sheets thinly coated in which crystallization tends to commence immediately upon exposure of the coating to the air.

5 One important advantage of the invention is that the necessity for heating the treating substance is eliminated, together with the consequent increased cost. Our treating substance may be applied at its natural storage or room 10 temperature and does not need to be heated. Apparently the very fine state of sub-division of the particles of the mist prevents the mist from having an undesirable cooling effect which might tend to buckle the sheet. Furthermore, the 15 resistance to corrosion of the coated product does not appear to be substantially lower than the resistance to corrosion of an ordinary spangled galvanized sheet, which is noted for being highly 20 corrosion resistant.

It is old to wipe the molten zinc coating applied to sheets by means of a steam jet. This does not, however, produce a product of the character in which we are interested. The effect of a jet of dry steam is to wipe the coating, while 25 the effect of a jet of wet steam is to make the coating brighter and more or less non-uniform. Also, a cooling air blast has been applied to galvanized sheets on emergence from a zinc bath, but this treatment does not produce the uniform 30 dull unspangled matte finish which we produce but rather tends to increase the brightness and spangled effect of the zinc coating. Our process does not result in wiping the coating and is effective on either light or heavy coatings.

35 While we have shown and described certain present preferred apparatus for and methods of carrying out our treatment, it is to be distinctly understood that the invention is not limited thereto and is of relatively wide application to 40 products other than sheets and may be otherwise variously embodied and practiced within the scope of the following claims.

We claim:

1. In the manufacture of metal coated products, the steps comprising applying to a base a molten zinciferous coating such as would upon cooling normally form crystals of large size commonly termed "spangles" and thereafter and while the coating is at least partially molten subjecting the coating to an atomized liquid mist the particles of which are sufficiently small to inhibit the propagation of crystals visible to the naked eye.

45 2. In the manufacture of metal coated products, the steps comprising applying to a base a molten zinciferous coating such as would upon cooling normally form crystals of large size commonly termed "spangles" and thereafter and while the coating is at least partially molten subjecting 50 the coating to an atomized mist of a solution of a chemical which forms a minute precipitate at about the solidification temperature of the coating metal and the particles of which are sufficiently small to inhibit the propagation of crystals visible to the naked eye.

55 3. In the manufacture of coated metallic sheets, the steps comprising applying to a base sheet a molten zinciferous coating such as would upon cooling normally form crystals of large 60 size commonly termed "spangles" and thereafter and while the coating is at least partially molten subjecting the coating to an atomized liquid mist the particles of which are sufficiently small to 65

70

75

inhibit the propagation of crystals visible to the naked eye.

4. In the manufacture of coated metallic sheets, the steps comprising applying to a base sheet a molten zinciferous coating such as would upon cooling normally form crystals of large size commonly termed "spangles" and thereafter and while the coating is at least partially molten subjecting the coating on one face only of the sheet to an atomized liquid mist the particles of which are sufficiently small to inhibit the propagation of crystals visible to the naked eye.

5. In the manufacture of metal coated products, the steps comprising applying to a base a molten zinciferous coating such as would upon cooling normally form crystals of large size commonly termed "spangles" and thereafter and during the early stages of crystallization of the coating sub-

jecting the coating to an atomized liquid mist the particles of which are sufficiently small to inhibit the propagation of crystals visible to the naked eye.

6. In the manufacture of metal coated products, the steps comprising passing the metal to be coated through a bath of a molten zinciferous coating material such as would upon cooling normally form crystals of large size commonly termed "spangles" whereby to coat the same and thereafter and while the coating is at least partially molten subjecting the coating to an atomized liquid mist the particles of which are sufficiently small to inhibit the propagation of crystals visible to the naked eye.

NELSON E. COOK.  
EDWARD J. KNOPF.  
WILLIAM L. DIEHL.